

# United States Patent

Susami et al.

[15] 3,660,973

[45] May 9, 1972

[54] SPUN YARN AND A METHOD FOR  
MANUFACTURING THE SAME

[72] Inventors: Kozo Susami; Keiichi Minami; Masaoaki  
Tabata; Teiyo Kojima; Zyuji Yunoki, all  
of Otsu-shi, Japan

[73] Assignee: Toray Industries Inc., Chuo-ku, Tokyo,  
Japan

[22] Filed: Sept. 29, 1969

[21] Appl. No.: 861,933

[30] Foreign Application Priority Data

Sept. 30, 1968 Japan.....43/70191  
Oct. 7, 1968 Japan.....43/72445  
Oct. 11, 1968 Japan.....43/73500  
Oct. 21, 1968 Japan.....43/76134  
Oct. 22, 1968 Japan.....43/76511

[52] U.S. Cl.....57/139, 57/58.95, 57/140 BY,  
57/156

[51] Int. Cl.....D02g 3/02, D01h 1/12

[58] Field of Search .....57/139, 140, 140 BY, 58.89,  
57/58.91, 58.93, 58.95, 156

[56]

References Cited

UNITED STATES PATENTS

|           |         |                   |            |
|-----------|---------|-------------------|------------|
| 2,911,783 | 11/1959 | Götzfried.....    | 57/58.95   |
| 3,126,697 | 3/1964  | Cizek et al.....  | 57/58.89   |
| 3,163,976 | 1/1965  | Juillard .....    | 57/58.95 X |
| 3,501,907 | 3/1970  | Tabata et al..... | 57/139 X   |
| 3,511,042 | 5/1970  | Seidov et al..... | 57/58.89   |
| 3,523,300 | 8/1970  | Tabata et al..... | 57/58.91   |

Primary Examiner—Stanley N. Gilreath

Assistant Examiner—Werner H. Schroeder

Attorney—Robert E. Burns and Emmanuel J. Lobato

[57]

ABSTRACT

A spun yarn having a particular internal configuration wherein the number of twists of the outer fibrous layer is different from that of the inner fibrous layer, spiral diameter of fibers composing the yarn is almost identical, unevenness index does not exceed 10 and variation coefficient of stretching tension is smaller than 4. In the manufacturing method, a particular relationship is established between the configurational feature of the supplied fiber bundle and the mechanical conditioning of the system.

6 Claims, 7 Drawing Figures



PATENTED MAY 9 1972

3,660,973

SHEET 1 OF 4



Fig. 2



PATENTED MAY 9 1972

3,660,973

SHEET 2 OF 4

*Fig. 3A*



*Fig. 3B*



Fig. 4



PATENTED MAY 9 1972

3,660,973

SHEET 4 OF 4

Fig. 5



Fig. 6



## SPUN YARN AND A METHOD FOR MANUFACTURING THE SAME

The present invention relates to an improved spun yarn and a method for manufacturing the same, more particularly it relates to a spun yarn having particular internal configurational features and a spinning method of an open-end-type for manufacturing the same utilizing pneumatic force.

The term "outer fibrous layers of a yarn" hereinafter used refers to fibrous layers of the yarn radially remote from a central longitudinal axis of the yarn while the term "inner fibrous layers of a yarn" hereinafter used refers to fibrous layers of the yarn radially in the vicinity of the central longitudinal axis. Be it understood that there is no distinct boundary between the above-defined two kinds of fibrous layers, and a fibrous layer radially interior to another fibrous layer is called as inner, with respect to the latter.

The term "a spiral diameter of a single fiber" hereinafter used refers to a diameter of a circle made by the spiral of the fiber taken along a direction perpendicular to a longitudinal central axis of the fiber.

The term "an unevenness index  $Z$ " hereinafter used refers to a value calculated in the following manner. A  $U_e$  percent of a spinning yarn is obtained by measuring unevenness of the yarn on an evenness Uster-type tester and a critical percent unevenness  $U_t \times 80/q$  is also calculated when "q" is a number of component fibers contained within a lateral cross-section of the yarn. Then, the unevenness index  $Z$  is given by

$$U_t \left( \frac{U_e^2}{U_t^2} - 1 \right).$$

The term "a variation coefficient of stretching tension  $S$ " hereinafter used refers to a value measured and calculated in the following manner. A spun yarn to be measured is passed through a zone intervening two pairs of rollers located apart from each other by 30 cm. The ratio of a surface speed of the downstream side roller, with respect to that of the upstream side roller, is set at 1.05. The tension of the spun yarn passed is successively measured by a suitable tension meter and recorded by a suitable recording device connected to the meter. Then, the variation coefficient of stretching tension  $S$  can be calculated from thus obtained record by using a conventional method.

In the conventional method of manufacturing a spun yarn, a plurality of single fibers of limited length are assembled together to form a fiber strand, the fiber strand is subjected to fiber orientation and stretching so as to have a desired thickness. Finally, a spun yarn of desired features can be acquired by imparting twists to this fiber strand. When a yarn manufacturing method of the above-described type is adopted, one cannot obviate the formation to an appreciable extent of unevenness in both yarn thickness and fluctuation in the yarn's mechanical properties due to the lengthwise positional relationship and arrangement of individual fibers composing the yarn.

Further, as is well-known, most of the spun yarn is used for making a fabric or a cord by passing them through several subsequent processes. Therefore, the above-described unevenness in yarn thickness often tends to effect lowering of the apparent quality of the end products made up of the yarns and the above-described fluctuation in the yarn's mechanical properties often tends to cause processing troubles, such as yarn breakages, in the subsequent processes resulting in lowering of the processability of the yarns used.

Many methods have been proposed for decreasing the above-described unevenness and fluctuation in the yarn characteristics. Increase in the strand doubling number is one of the attempts and use of two-folded yarns is another of the attempts. However, none of the conventional attempts could provide a sufficient solution to the problem of unevenness of spun yarns while problems still remained to be solved in the field of textile industry.

Generally, synthetic fibers lack in hygroscopic property and, because of this reason, they are not suitable for uses which require superior hygroscopic property such as pile

fabrics purposed for undershirts, towels or bedsheets. In order to supplement this poor hygroscopic property of the synthetic fibers, they are usually blended with wool, cotton, or regenerated fibers. Another attempt in this regard consists in formation of a large number of fine spaces in the yarn configuration so as to utilize capillarity effect due to presence of such fine spaces. In case the product is used for undershirts, a comfortable feeling of the product to the human skin is also required. The word comfortability is a totalized conception of hygroscopic property, water absorptiveness, drape, hand feeling and air permeability of the product. Among the listed properties, softness, bulkiness, hygroscopic property and water absorptiveness are particularly of great importance. Thusly, as a marketable product, the spun yarn requires excellent softness, bulkiness, hygroscopic property, water absorptiveness, drape and air permeability together with increased adaptability for a weaving process. In this connection, however, it is actually very difficult to provide a spun yarn composed of hydrophobic fibers, especially of synthetic fibers, will all the above-listed properties in a completely balanced condition.

A principal object of the present invention manufacturing a spun yarn having less unevenness in its thickness and uniform mechanical properties along the lengthwise direction thereof together with an enhanced adaptability for subsequent processes for making end products.

Another object of the present invention is to manufacture a spun yarn of excellent bulkiness and hygroscopic property from so-called hydrophobic material fibers.

A further object of the present invention is to manufacture a sliver used for making spun yarns of the above-described features.

A still further object of the present invention is to provide a novel spinning method of an open-end-type for manufacturing a spun yarn of the above-described nature utilizing pneumatic force.

In conformity to the above-described objects, the spun yarn of the present invention is provided with the following characteristic configurational features. In the yarn configuration, the number of twists of the outer fibrous layer is different from that of the inner fibrous layer with respect to the central longitudinal axis of the yarn. The spiral diameter of every fiber composing the yarn is almost identical. Further, the value of the unevenness index  $Z$  does not exceed 10 while the value of the variation coefficient of stretching tension  $S$  does not exceed 4.

As before mentioned, the yarn manufacturing method of the present invention is essentially a kind of so-called open-end-type spinning system. Fibers are supplied to a feeding device through a pair of feed rollers in the form of a fiber strand. Being introduced into the feeding device, the individual fibers are liberated from the bundle during their transportation to a downstreamly disposed rotor. In this fiber liberating mechanism, the method of the present invention preferably utilizes a pneumatic force created by a compressed air supply. The liberated fibers are ejected and accumulated onto an inside wall of the rotor and adheres thereon due to a centrifugal force caused by the high speed rotation of the rotor. Next, the adhered fibers are removed therefrom in a rebundled condition and delivered out of the rotor while being twisted to have a form of a spun yarn.

As a result of intensive study on the drawbacks encountered in the use of the prior art, the inventors of the present invention have revealed that unevenness of a yarn thickness has a close relationship to its effects on subsequent processes and final products made up of the yarns and that both of production efficiency in the processes and quality of the final products can be remarkably enhanced if the above-defined unevenness characteristics fall within a certain area of value. From this viewpoint, they tried to pick up the above-described values  $Z$  and  $S$  as the yarn unevenness characteristics to be defined and confirmed that a spun yarn having configurational features defined by  $Z$  smaller than 10 and by  $S$  smaller than 4.0 is optimum for attaining the objects of the present invention.

tion. By thus defining the configurational features of the spun yarn, the art of the present invention eliminates the need of folding two or more single spun yarns resulting in effective art of surplus textile production expense. Further, the art of the present invention is effective in enrichment of relatively poor bulkiness characteristic to the conventional spun yarns, that is, the spun yarn of the present invention is provided with preferable softness and excellent resiliency.

The spun yarn of the above-described nature can hardly be manufactured by any of the conventionally known spinning systems of ring-spinning type. In the yarn spinning mechanism of these types, a roving is subjected only to a lengthwise drafting operation and unevenness in the roving thickness survives, although its lengthwise period is elongated due to the drafting, in the resultant configuration of the formed spun yarn. The unevenness index still remains at a high level and the variation coefficient of stretching tension still remains at a remarkably high level. This is a fatal drawback of the ring-spinning system and elimination of such trouble may be achieved only by completely reforming or revolutionally converting the spinning mechanism of this type.

In connection with this, the inventors of the present invention have come to a conclusion that the spun yarn concerned with the present invention can be effectively manufactured by employing an extremely high drafting together and simultaneously with a large extent of doubling in the process from a roving to a spun yarn and they established the above-defined method for manufacturing the novel spun yarn of the present invention. The spun yarn manufactured by this method is configurationally characterized in that the number of twists of outer fibrous layers is different from that of inner fibrous layers with respect to a central longitudinal axis of the yarn and the spiral diameter of every fiber composing the yarn is almost identical. As is well understood from this particular twist configuration, there is no interference among the actions of the fibers composing different fibrous layers. This means that reaction of the outer fibrous layer against bending or torsional deformation externally applied to the yarn is independent from that of the inner fibrous layer. That is, less inter-fiber frictional contact takes place within the yarn configuration even at twice such deformations.

It is well-known that the inter-fiber frictional contact dominates the resiliency of the yarn against applied deformations of small extent. So, the spun yarn of the present invention is provided with excellent resiliency together with increased softness due to less inter-fiber frictional contact against applied deformations of the above-described nature. None of the conventional ring-spinning systems can provide the spun yarn having such excellent mechanical properties.

In addition to the above-described definitions, the yarn manufacturing method of the present invention further requires additional definition concerning the nature of a fiber strand to be supplied to the system.

Mechanical relationship between individual fibers contained in the supply fiber strand and air flow used in the open-end-spinning system of the present invention will be hereinafter explained. Drawing our attention to a single particular fiber contained in the supplied fiber strand, a trailing end portion of the fiber is nipped by a pair of feed rollers at the beginning and is released therefrom as the supply goes on. After this releasing from the nip, the particular fiber tends to be maintained within the fiber strand due to frictional contact with other fibers surrounding that particular fiber in the fiber strand. Together with this, that particular fiber is placed under the effect of the air flow advancing through the feeding device of the system and tends to be liberated from the fiber strand due to frictional contact with the advancing air flow. The relationship between the frictional force for maintaining that particular fiber in the fiber strand (hereinafter referred to as "Draw-out resisting force") and the pneumatic frictional force for liberating that particular fiber from the fiber strand (hereinafter referred to as "Keep-in resisting force") changes from time to time after the relief of the fiber strand from the nip by the feed rollers.

Just after the particular fiber is released from the nip by the feed rollers, the draw-out resisting force exceeds the keep-in resisting force by the advancing air flow and the particular fiber is maintained in the fiber strand. As time goes on, the former becomes smaller than the latter and the particular fiber can be liberated from the fiber strand. This fiber liberating mechanism is essential in carrying out the yarn manufacturing method of the present invention with optimum results.

The above-described fiber liberating operation can be regarded as a kind of fiber strand drafting operation. From this view point, fibers whose trailing end is caught by the feed rollers can be referred to as "low speed fibers", fibers released from the catch but still maintained in the fiber strand can be referred to as "floating fibers" and fibers completely liberated from the fiber strand into the air flow can be referred to as "high-speed fibers". Our knowledge of conventional drafting mechanism teaches us the fact that less quantity of the floating fibers brings about more uniform drafting effect. This discussion can also be applied to the open-end-type spinning system of the present invention, that is, the less floating fibers in the feeding device of the present invention, the smaller the unevenness of the resultant yarn thickness and the fewer occurrences of accidental yarn breakage. With increase in the quantity of the floating fibers within the feeding device, non-uniformity tends to take place in the drafting operation performed by the feed roller and the fiber liberating air flow. This tends to disturb uniform and stable supplying of liberated fibers into the spinning rotor resulting in formation of unfavorable unevenness of yarn thickness and frequent chances of yarn breakage.

Basing upon a profound study of the above-explained fiber liberating mechanism, the inventors of the present invention succeeded in providing a method for effectively liberating individual fibers from the supplied fiber strand and instantly changing them to high-speed fibers while suitably dominating formation of the floating fibers. This can be attained by defining the relationship between the draw-out resisting force  $F_D$  and the keep-in resisting force  $F_A$ , both in mg scale, as follows.

$$F_A - (F_D/NL) > 0.45$$

wherein,

$N$  = Number of individual fibers contained in a lateral cross-section of a fiber strand supplied to the system.

$L$  = Average fiber length in mm scale.

When the process characteristics have the above-defined relationship to the nature of the supplied fiber strand, the fiber supplied to the spinning rotor can be carried out in a stable and uniform condition assuring decrease in yarn breakage and yarn unevenness.

Measuring methods of the above-described draw-out and keep-in resisting forces  $F_D$  and  $F_A$  will hereinafter be illustrated.

The draw-out resisting force  $F_D$  is measured using a fiber strand of 0.5 T.P.I. and 90 gram/yarn. The fiber strand is nipped at two points apart from each other by a distance twice the average fiber length of the strand and at one of the nip points, the strand is drawn remotely away from the other nip point into a longitudinal direction thereof at a drawing rate of 20 mm/min. At this stage of the fiber strand drawing operation, maximum values of the draw-out resisting force are measured twenty times and the measured results are calculated into the draw-out resisting force  $F_D$  in mg.

The keep-in resisting force  $F_A$  is measured in the following manner. Five single fibers are bundled with their one ends arranged in order. A bundle portion extending from the arranged end by 15 mm is exposed into an air flow advancing at a speed of 11 m/sec., the keep-in resisting force in this condition is measured twenty times and the keep-in resisting force  $F_A$  in mg is obtained by dividing an average of thus measured values by 75.

As is already explained, in the open-end spinning system, less quantity of the floating fibers within the feeding device will lead to a smaller extent of yarn unevenness and less occurrence of yarn breakage. Be it noted, that the quantity of the floating fibers within the feeding device is dependent upon the

values of draw-out resisting force  $F_D$  and keep-in resisting force  $F_A$ . The smaller the value of the former and the larger the value of the latter, the lesser the quantity of floating fibers. This is because, as is already explained, production of the floating fibers is dependent upon the relationship between the extent of the frictional force applied to floating fibers by the surrounding fibers in the fiber strand supplied into the feeding device and the extent of the pneumatic frictional force applied to the floating fibers by the advancing air flow. When the former is larger than the latter, the floating fibers cannot be converted into high-speed fibers. The conversion takes place only when the latter exceeds the former.

From the foregoing discussion, it is apparent that the draw-out resisting force  $F_D$  is representative of the frictional force applied to the floating fibers by the surrounding fibers while the keep-in resisting force  $F_A$  is representative of the pneumatic frictional force applied to the floating fibers by the advancing air flow within the feeding device. Therefore, the difference between  $F_A$  and  $(F_D/NL)$  should preferably be larger than a certain value and the value was confirmed by the inventors of the present invention to be 0.45. By defining the relationship between  $F_D$  and  $F_A$  in this way, a remarkable decrease in yarn breakage and yarn unevenness can be realized.

In addition to the foregoing discussion, it was also confirmed by the inventors of the present invention, that configurational characteristics of staple fiber composing a supplied sliver gave an important repercussion upon the fiber transporting, liberating and orienting function of the spinning system. As one such configurational characteristics, cross-sectional profile characteristic  $K$  was selected and critical values thereof were experimentally investigated.

The characteristic  $K$  can be measured and calculated in the following manner.

Provided that a staple fiber has a fineness of  $d$  denier and a specific gravity of  $\rho$  g/cm<sup>3</sup>, that each fiber has a columnlike shape of uniform diameter and that the cut cross-sectional area of each fiber is negligible, then the total surface area  $\delta$  m<sup>2</sup>/g of 1 g of stable fibers is given by

$$\delta = 0.3363 \frac{1}{\sqrt{d \cdot \rho}}$$

Whereas, most of the actual fibers are not provided with column-like shape of uniform diameter and the cross-sectional profile thereof is mostly deviated from round. Therefore, the actual value of the total surface area of 1 g of fibers is larger than the  $\delta$ -value calculated by the above formula. The difference between thus calculated  $\delta$ -value and the value of the actual value of the total surface area can be an index of the deviation of the cross-sectional profile from round.

It is well-known that the fineness  $d_A$  in  $\mu\text{g}/\text{inch}$  measured on a micronaire is in inverse proportion to the square value of the total surface area  $\delta A$  of a definite quantity of fibers as follows.

$$d_A = (K_0 / \delta A^2)$$

where

$K_0$  = constant.

The micronaire fineness  $d_A$  is measured by applying 6 lbs/inch<sup>2</sup> pneumatic pressure to 3.24 g, fibers on the micronaire and the characteristic  $K$  is calculated as follows.

$$K = d_A \cdot \delta^2 / \delta_A^2$$

$$= K_0 \cdot \delta^2 / \delta_A^2$$

$$= 0.113 (d_A / \rho)$$

Thus, the characteristic  $K$  represents the deviation of the cross-sectional profile of the fiber from round and the value of the characteristic  $K$  decreases with increase in the total surface area of 1 g fibers. The value of  $K$  for a polyester fiber having a nearly round cross-section is 0.326 and the value for a rayon fiber having a complete cross-sectional profile is 0.292.

In the open-end spinning system utilizing pneumatics, the less the quantity of floating fibers in the fiber feeding device, the smaller the extent of the resultant yarn unevenness and the occurrence of yarn breakage. This quantity of floating fibers is dependent upon the relation between the frictional force for keeping the fibers within the supplied fiber bundle and the

70  
75

pneumatic force tending to draw those fibers out from the bundle into the pneumatic flow. As the latter becomes larger than the former, the quantity of the floating fibers decreases accordingly. Therefore, production of a spun yarn of enhanced quality in a stable processing condition can be attained if a bundle of fibers having a keep-in resisting force far larger than a draw-in resisting force is desirably supplied to the production system. The difference between the above-described both forces has a direct relationship to the cross-sectional profile of the fibers. Hence, it will be well understood that the above-mentioned characteristic  $K$  has an important significance in the art of the open-end spinning system of the present invention.

Further features and advantages of the art of the present invention will be more apparent from the ensuing description, reference being made to the accompanying drawings; in which

FIG. 1 is a skeleton sketch of a preferred embodiment of a spinning system for carrying out the method of the present invention,

FIG. 2 is a graphical drawing for presenting a relationship between  $A$  and the mechanical condition of the yarn manufacturing system,

FIGS. 3A and 3B are graphical representations of lengthwise fluctuation in stretching tension of yarns manufactured by the method of the present invention and the ordinary ring-spinning method, respectively,

FIG. 4 is a graphical representation of relations between twist constant, tensile strength and percent water retainment of the yarn manufactured by the method of the present invention,

FIG. 5 is an explanatory drawing for showing a method of measuring bending strength of single fibers,

FIG. 6 is a graphical drawing for showing a relation between bending strength of the material fiber and the degree of bulkiness of the resultant product made by the method of the present invention.

Referring to FIG. 1, a preferred embodiment of the spinning system for carrying out the method of the present invention is shown. A fiber strand 1 is supplied from a given draft mechanism (not shown) to a feeding device 3 through a pair of feed rollers 2a and 2b being sucked thereto by a pneumatic suction force due to a compressed air supply. By the operation of this pneumatic force, the fibers contained in the supplied fiber strand are liberated therefrom, transported pneumatically through the feeding device and ejected against an inside peripheral wall of a spinning rotor 4 through an outlet termination of a delivering pipe 6 of the feeding device 3 directed thereto. The spinning rotor 4 rotates at an extremely high rotating speed around its vertical central axis and the introduced fibers adhere to the spinning rotor's inside wall and, in this adhered condition, rotate around the central axis due to centrifugal force caused by the high speed rotation of the spinning rotor 4. Then, the fibers are removed therefrom in succession, rebundled while being twisted on its path from the removal point to the bottom rotary axis 7 of the opening rotor 4, delivered out of the rotor 4 through the bottom rotary axis 7 in the form of a spun yarn 8 and taken-up in the form of a package 9 by a pair of take-up rollers 11a and 11b and a winding drum 12 to which the package 9 peripherally contacts.

The manufacturing mechanism of the spun yarn of the present invention in the above-described spinning system is as follows. Now, provided that the supplied fiber strand 1 has unevenness of thickness of sine-wave-like profile defined by a wave-length " $\lambda$ " and a relative amplitude " $a$ ", the thickness of the fiber strand  $S(X)$  at the location  $X$  on the yarn longitudinal axis is given by;

$$S(X) = \bar{S} \left( 1 + a \sin \frac{2\pi}{\lambda} X \right) \quad (1)$$

Being delivered from the draft equipment, the fiber strand is subjected to a draft operation at a draft ratio of  $(V/U)$  provided that the delivery speed of the strand from the draft equipment is  $U$  and the surface speed of the rotating spinning

rotor inside wall is  $V$ . As a result of this draft operation, the average thickness of the fiber strand becomes as  $\bar{S} \cdot \bar{U}/V$  and the thickness  $S(X)$  of the fiber strand at the location  $X$  is given by;

$$S(X) = \frac{\bar{U}}{V} \bar{S} \left( 1 + a \sin \frac{2\pi}{\lambda} X \right) \quad (2)$$

wherein

$$\lambda = (\lambda N / \bar{U})$$

Provided that the spun yarn is taken up at a speed  $W$ , the fiber strand of this nature is given by  $Q = V/W$  times accumulated on the rotor's inside wall and the unevenness of thickness  $S'(X)$  thereof is given by;

$$S'(X) = \frac{\bar{S} \cdot \bar{U}}{W} \left\{ 1 + a A \sin \frac{2\pi}{\lambda} \left( X + \frac{(Q-1)l}{2} \right) \right\} \quad (3)$$

wherein

$l$  = One peripheral length of the spinning rotor inside wall and

$$A = \frac{\lambda W}{\pi l \bar{U}} \sin \frac{\pi l \bar{U}}{\lambda W} \quad (4)$$

A relation between  $A$  and the mechanical condition of the system is graphically shown in FIG. 2. In general cases, the value of  $(LU/\lambda/\lambda W)$  exceeds 1 and, therefore, the value of  $A$  is smaller than one-fifth. This means that the amplitude of the unevenness possessed by the supplied fiber bundle, which can be regarded as corresponding to the unevenness of yarn thickness in the ordinary ring-spinning system, can be decreased to smaller than one-fifth of it by processing through the spinning system of the present invention provided that no additional unevenness creation takes place in the feeding device. Therefore, it is concluded that an adequate and optimum combination of the raw fibrous material selection and the feeding device conditioning can successfully provide a spun yarn having extremely decreased extent of unevenness comparing to the conventional type spun yarns.

On the other hand, lengthwise fluctuation of the spun yarn's mechanical properties, such as the variation coefficient of stretching tension, are affected by the unevenness of thickness and twist-configuration of the yarn. So, the mechanical properties' fluctuation of the yarn of the present invention is expected to be relatively small because of its small unevenness of thickness. Further, the particular twist configuration possessed by the yarn of the present invention has a great significance in decreasing the value of the variation coefficient of stretching tension of the yarn.

As the result of the repeated experimental test, it was confirmed that, in the case of the spun yarn of the present invention, the ratio of the variation coefficient of stretching tension  $S$  with respect to the corresponding value of the unevenness index  $Z$  ranges in between 0.25 and 0.50 and is far smaller than that of the yarn manufactured by the conventional ring-spinning method, which is ordinarily larger than 0.50. This will be well understood by comparing the results shown in FIGS. 3A and 3B. In the example shown in FIG. 3A, a polypropylene 100 percent spun yarn of 30<sup>s</sup> (cotton spinning count), manufactured by the method of the present invention, is used for measuring the lengthwise fluctuation in stretching tension, taken on the ordinate, while a same yarn manufactured by the ordinary ring-spinning method is illustrated in FIG. 3B.

Basing upon the above-presented experimental observation, the reason for the small variation coefficient of stretching tension in the yarn of the present invention is estimated as follows.

It is theoretically assured that not only the measured unevenness of thickness but also the essential unevenness of thickness inherent in the spun yarn of the present invention is smaller than those characteristic to the conventional spun yarns. In addition to this, as is already discussed, the fibers contained in the inner fibrous layers having fiber twists respond to the external tensile force applied to the yarn while the fibers in the outer layers having more twists present little

reaction to this force application. This means that only the fibers in the fibrous layers having smaller unevenness of thickness are mainly responsible for the tension designation measured in the test. This is the reason that the variation coefficient of measured stretching tension is remarkably smaller in its extent than the unevenness of yarn thickness is.

The spun yarn of the above-described excellent nature can be obtained in the open-end-type spinning system of the present invention by using a material fiber strand containing natural fibers such as cotton, wool and silk, regenerated fibers or synthetic fibers. Synthetic fibers of extremely hydrophobic nature can also be used as the material. Especially, when synthetic fibers having a moisture content of 4 percent or smaller is used as the material, the resultant spun yarn can be provided with uniform distribution of fine voids in the all-fibrous configuration thereof and an excellent humidity absorptiveness represented by a "percent water retention" of 150 or more.

The term "moisture content" above-used refers to that inherent in a single fiber in a condition of 20° C and 65 percent relative humidity and the value is given in the form of an average of the moisture contents possessed by the respective fibers.

The measure "percent water retention" above-used is obtained in the following manner. The specimen spun yarn is taken up in the form of a skein for 100 times on a reeling machine having a peripheral length of 1 m. After being immersed into water of 20° C for 20 minutes, the skein is hung by its one end, for the purpose of water removal, within a room conditioned at 20° C and 65 percent relative humidity. When water ceases to drop from the skein, the weight  $W$  of the skein was measured. Then, provided that the weight of the skein within a room of 20° C and 65 percent relative humidity before water immersion is given by  $W_0$ , the percent water retention of the specimen fiber is given by;

$$(W - W_0/W) \times 100$$

The measure "apparent percent boiling water shrinkage" hereafter used, is measured in the following manner. A single fiber is immersed in a boiling water bath in a relaxed condition for 20 minutes and left for approximately a whole day in this relaxed condition within a room conditioned at 20° C and 65 percent relative humidity for the purpose of drying. After drying, the specimen fiber is subjected to a 2 mg/denier loading and the resultant percent shrinkage is calculated from thus obtained experimental results.

The measure "true percent boiling water shrinkage" hereafter used is measured by preparing a dried specimen fiber in the same manner as explained above. This prepared specimen fiber is next subjected to a 300 mg/denier loading and the obtained result is calculated into the true percent boiling water shrinkage.

The hydrophobic synthetic fiber preferably used in the art of the present invention should have a percent boiling water shrinkage of 5 or smaller together with a moisture content of 4 percent or smaller and such synthetic fibers as polyacrylonitriles, polyesters, polyamides and polypropylenes can favorably conform to this requirement. It is preferable that the fibrous material used in the art of the present invention should contain 30 percent by weight or more hydrophobic fibers as its component.

As is already-described, the internal configuration of the spun yarn thus prepared is characterized by being provided with numerous fine voids uniformly distributed in the respective fibrous layers. This uniform distribution of numerous fine voids is brought about because, in the spinning system of the present invention, pneumatically liberated individual fibers are rebundled due to centrifugal force and vortical air flow created inside the spinning rotor. This presence of numerous fine voids provides the yarn of the present invention with remarkably large humidity absorptiveness due to capillarity. So, even when hydrophobic fibers occupy a major part of the material fibers, the resultant spun yarn can be provided with superior humidity absorptiveness as compared to that of the conventional spun yarns made up of hydrophobic fibers.

In this connection, however, even in the case of an open-end spinning system, impartation of hard twists decreases the number of voids resulting in lowering of the water retainability of the yarn while impartation of slight twists tends to lower the resultant yarn tensile strength resulting in frequent yarn breakages and fluff formation in the subsequent processes and lowering of the end products' quality. Spun yarns of 20 to 40° (cotton count system) are favorably adapted for uses requiring humidity absorptiveness.

Referring to FIG. 4, relations between the twist constant, the yarn tensile strength and the percent water retainment are graphically shown. In the drawing, symbols ● and the solid line are for the relation between the twist constant and the percent water retainment while symbols ○ and the dotted line are for the relation between the twist constant and the product of the yarn count and the yarn tensile strength. As is apparent from the results shown in the drawing, the percent water retainment decreases as the value of the twist constant increases while the above-described product also decreases as the value of the twist constant becomes smaller than 4.0. Taking both tendencies into consideration together, the value of the twist constant preferably employable in the art of the present invention resides in between 3.5 and 5.0. Although polyacrylonitrile fibers of 1.5<sup>d</sup> × 38 mm were used as the specimen in the above experiment, it was confirmed that similar results could be achieved even if other type fibers were used.

Next, how the quality of the resultant product is affected by the twist constant and the percent water retainment of the material spun yarn will be discussed.

Specimen undershirts were made up of the following three types of sample yarns by a knitting manner and were subjected to a performance test the result of which is illustrated in Table 1.

Sample I: A spun yarn of synthetic fibers manufactured by the ordinary ring-spinning-type method.

Sample II: A spun yarn made by the method of the present invention.

Sample III: A bulky yarn made by blending highly shrinkable fibers with low shrinkable fibers.

TABLE 1

| Sample   | Percent water retainment | Result of performance test                                                                                                                                                                                                                                        |
|----------|--------------------------|-------------------------------------------------------------------------------------------------------------------------------------------------------------------------------------------------------------------------------------------------------------------|
| I.....   | {150 or (smaller         | {Less presence of fine voids in the fabric configuration results in smaller humidity absorptiveness due to capillarity. Uncomfortable and hard touch were objected to. Only 4 out of 100 examiners felt comfortable.                                              |
| II.....  | {150 or (more            | {Moderate extent of voids present in the fabric configuration assures excellent humidity absorptiveness such as sweat. Medium softness accompanied by rich resiliency presents comfortable feeling to human skin. Up to 75 out of 100 examiners felt comfortable. |
| III..... | {Not definite            | {Small humidity absorptiveness once excessive softness. Suitable especially for baby wear. 21 out of 100 examiner's felt comfortable.                                                                                                                             |

As is apparent from the results shown in the table, an undershirt having preferable humidity absorptiveness, softness moderately combined with resiliency can be obtained if percent water retainment of the material yarns becomes 150 or more. The sample yarn III can also possess such degree of percent water retainment. However, the percent shrinkage of the highly shrinkable fiber must be 5 or more, more generally from 15 to 30, in order to manufacture a high bulky yarn of this nature and this is out of the technical scope of the present invention.

Next, using various fibers listed in Table 2 as the material, several fiber strands were prepared. Next, the prepared fiber strands were processed through the open-end spinning system of the present invention and the ring-spinning system of the conventional type. The resultant yarn count was 24° for both cases and the twist constants were 4.2 for the former and 3.6 for the latter. Thus manufactured spun yarns were taken up in the form of skeins in a manner above-described and were sub-

jected to measurement of percent water retainment, the results of which are illustrated in Table 3.

TABLE 2

| Sample number | Kind of fiber used     | Fineness in denier fiber length in mm. | Percent moisture content at 20° C. temperature and 65% relative humidity |
|---------------|------------------------|----------------------------------------|--------------------------------------------------------------------------|
| A.....        | Polyacrylonitrile..... | 1.5×38                                 | 1.2~2.0.                                                                 |
| B.....        | Polyester.....         | 1.5×38                                 | 0.4~0.5.                                                                 |
| C.....        | Polyamide.....         | 1.5×38                                 | 3.5~5.0.                                                                 |
| D.....        | Polypropylene.....     | 1.5×38                                 | 0.                                                                       |
| E.....        | Rayon.....             | 1.5×38                                 | 12.0~14.0.                                                               |
| F.....        | Peruvian cotton.....   | 1.5×38                                 | About 7~8.                                                               |

Although the fineness of the fibers used in the present invention is selected according to the required count of the resultant spun yarn and to the end use of the product, it is generally and preferably in a range between 1.5 and 2.5 denier. The material fiber may be provided with three-dimensional crimps for the purpose of bulkiness impartation to the resultant yarn. However, provision of such crimps is not recommended in the art of the present invention because it sometimes requires increase in the yarn manufacturing cost and it tends to provide the resulting yarn with an apparent shrinkage exceeding 5 percent.

TABLE 3

| Sample No. | Manufacturing method fibers used | Material    | Resultant percent water retainment |
|------------|----------------------------------|-------------|------------------------------------|
| 1          |                                  | A           | 166.0                              |
| 2          |                                  | B           | 171.8                              |
| 3          | Present                          | C           | 175.2                              |
| 4          | inventions                       | D           | 176.1                              |
| 5          | system                           | E           | 212.8                              |
| 6          |                                  | A30%:E 70%  | 197.0                              |
| 7          |                                  | B 65%:E 35% | 173.9                              |
| 8          |                                  | A           | 140.6                              |
| 9          |                                  | B           | 111.6                              |
| 10         | Conventional                     | C           | 130.0                              |
| 11         | ring-                            | D           | 131.5                              |
| 12         | spinning                         | E           | 189.1                              |
| 13         |                                  | A30%:E 70%  | 161.5                              |
| 14         |                                  | B 65%:E 35% | 123.7                              |

The results presented in the table show us the fact that the open-end-type spinning system of the present invention can provide the resultant spun yarns with the percent water retainment of 150 or more, while in the case of the conventional spinning system of a ring-spinning-type, the value cannot exceed 150 especially when synthetic fibers are solely used. (See the rows of A, B, C and D.)

Having the above-described configurational characteristic features, the spun yarn of the present invention can be provided with lengthwise uniformity in various senses and, even when it is made up of synthetic fibers only, excellent humidity absorptiveness. Therefore, the spun yarn of the present invention is advantageously used as a material for undershirts, bedsheet, towels and socks assuring provision of excellent quality and soft hand feeling.

Further, these textile products have excellent resistance against abrasion and pill-formation during practical use. For this purpose, the fibers composing the fiber strand need to have a bending strength of 400 times or larger. By using a fiber strand made up of fibers having such a bending strength, the resultant textile products will have a degree of bulkiness ranging between 6.0 and 7.0 cm<sup>3</sup>/g and, within the range of this degree of bulkiness, they can have remarkably enhanced resistances against abrasion and pill-formation during actual use thereof.

The above-described measure "bending strength" is obtained in the following manner, reference being made to FIG. 5. A single fiber 13 is crossed with another single fiber 14 with their including angles  $\alpha$  and  $\beta$  being 60° in such a manner that

a plane defined by the vent fiber 13 crosses with that defined by the bent fiber 14 at right angles. Two ends of the fiber 14 are fixed to a pair of rods 16 secured onto a plate 17, which is swung from its horizontal position by 15°. One end of the fiber 13 is fixed to a stationary point and another end of it is connected to a load 19 of 200 mg/denier passing over a rotatable roll 18 as shown in the drawing. By the swinging of the plate 17, the two fibers 13 and 14 are abraded with each other at their crossed contact and, with repetition of the abrasion, one of the fibers 13 and 14 will break down. Both of the specimen fibers 13 and 14 should be of the same kind and the number of abrasion repetitions at this moment of the fiber's break is referred to as the bending strength of that fiber. The bending strengths thus measured of several textile fiber yarns are as follows.

|                    |                   |
|--------------------|-------------------|
| Peruvian cotton    | from 600 to 1000  |
| Wool               | from 100 to 400   |
| Nylon              | larger than 10000 |
| Polyacrylonitrile  | from 100 to 300   |
| Polyester          | from 2000 to 4000 |
| Improved polyester | larger than 300   |

Therefore, in the art of the present invention, it is desirable to use fibers having a bending strength of 400 or larger, for example cotton, nylon or polyester fibers, and the fiber strand to be supplied to the open-end-type spinning system should preferably contain at least 30 percent by weight of fibers of such nature. In order to provide the resulting textile products with a degree of bulkiness ranging in between 6.0 and 7.0 cm<sup>3</sup>/g using the material spun yarns of the above-described nature, it is necessary to make the twist constant of the yarn from 4.0 to 5.5. The above-described bending strength of the material fiber and the degree of bulkiness of the resultant product have a close relationship to the resistances of the product against abrasion and pill-formation. This relationship will now be explained taking the case of socks as an example, reference being made to FIG. 6. In the drawing, bending strength in times of the material fiber is taken on the abscissa while resistance of the product against pill-formation in grade is taken on the ordinate. A shaded area "A" corresponds to the case of the conventional ring-spinning system while a shaded area "B" corresponds to the case of the open-end spinning system of the present invention. In the case of the conventional ring-spinning system, resistance against pill-formation can be higher than grade 3 when the bending strength is smaller than 300. However, the bending strength smaller than 300 tends to be accompanied by considerably lowered abrasion resistance as shown in Table 4. In contrast to this, the spun yarn of the present invention is characterized in that the resistance against pill-formation is not lowered even when the bending strength becomes larger than 400. Further, it is apparent from the results shown in the table that the abrasion resistance increases as the bending strength exceeds 400. Therefore, in the art of the present invention, it is preferable to make the bending strength of the material fibers larger than 400.

larger than 7.0 cm<sup>3</sup>/g, it also accompanies poor resistance against pill-formation.

TABLE 5

| Degree of bulkiness in cm <sup>3</sup> /g larger than | Result                                                                    |                                                                                                                                    |
|-------------------------------------------------------|---------------------------------------------------------------------------|------------------------------------------------------------------------------------------------------------------------------------|
|                                                       | Hard and undesirable touch. Only 16 out of 100 examiners liked the socks. |                                                                                                                                    |
| 10 7.0                                                | in between 6.0 and 7.0                                                    | Moderate softness with excellent comfortability and humidity absorptiveness. 58 out of 100 examiners feel the socks as preferable. |
| 15                                                    | larger than 7.0                                                           | Soft feeling and nice fit to wear but poor resistance against pill-formation. 26 out of 100 examiners feel the socks desirable.    |
| 20                                                    |                                                                           |                                                                                                                                    |

As is apparent from the above results, socks having excellent resistance against pill-formation, abrasion resistance, hand-feeling and bulkiness can be obtained only by employing the yarn manufacturing method of the present invention.

The following examples are illustrative of the art of the present invention, but are not to be construed as limiting the same.

## EXAMPLE 1

Spun yarns of the present invention (Sample Nos. 1, 2, 4 and 5) and spun yarn manufactured by the conventional ring-spinning system (Sample Nos. 3 and 6) were prepared and subjected to the following evaluation tests.

U percent and the unevenness index Z were measured on these prepared specimen yarns and fabrics of the following specification were woven from the specimen yarns.

Warp Polyester filament yarn  
 Filling Sample No. 1 Polyester 65 percent/Rayon 35 percent 20° Sample No. 2 Polyacrylonitrile 100 percent 20°  
 Sample No. 3 Polyester 65 percent/Rayon 35 percent 20°  
 Density Warp 100 end/inch Filling 65 pick/inch  
 Texture Plain weave

After the fabric formation, evaluation of the fabric appearance was also performed and the results are shown in Table 6.

TABLE 6

| Sample No. | U%   | Z    | Appearance                       |
|------------|------|------|----------------------------------|
| 1          | 9.8  | 9.95 | marketable in a particular field |
| 2          | 9.4  | 8.8  | marketable                       |
| 3          | 11.0 | 14.2 | not marketable                   |

TABLE 4

| Manufacturing system:                      | Ring-spinning system |      |         | Present invention's system |      |      |
|--------------------------------------------|----------------------|------|---------|----------------------------|------|------|
|                                            | 2,800                | 500  | 200     | 2,800                      | 500  | 200  |
| Bending strength                           | 2,800                | 500  | 200     | 2,800                      | 500  | 200  |
| Twist angle in degree                      | 52.0                 | 22.5 | 52.0    | 22.5                       | 52.0 | 22.5 |
| Degree of bulkiness in cm <sup>3</sup> /g  | 5.82                 | 6.32 | 5.76    | 6.21                       | 5.78 | 5.08 |
| Resistance against pill-formation in grade | 2.0~2.3              | 1    | 2.0~2.3 | 1                          | 4    | 3    |
| Abrasion resistance in times               | 650                  | 380  | 420     | 315                        | 216  | 181  |

With respect to the degree of bulkiness, it is well-known from the results shown in Table 5 that a comfortable feeling of the socks can be obtained if the degree of bulkiness is in a range between 6.0 and 7.0 cm<sup>3</sup>/g and that a hard and undesirable touch results when it is smaller than 6.0 cm<sup>3</sup>/g. Although a soft and desirable touch of the socks is obtained when it is

70 Appearance evaluation was performed through a see-through inspection by an expert inspector. It is concluded from this result that the unevenness index Z should preferably be smaller than 10, or more particularly smaller than 9.

75 Next, the variation coefficient of stretching tension S of various specimen yarns was measured and a relation between

the processability of the yarn and thus measured *S*-value was investigated. It is well-known by persons engaged in the art that the lengthwise fluctuation of mechanical properties of a textile yarn tends to cause lowering of production efficiency of textile products made of the textile yarns and deterioration of product quality. As an example, the relation between the *S*-value of a yarn and the frequency of yarn breakages in a weaving process using the yarn is illustrated in Table 7.

TABLE 7

| Sample No. | Material fibers            | Yarn count      | <i>S</i> in % | Yarn breakage in end/hr. loom |
|------------|----------------------------|-----------------|---------------|-------------------------------|
| 4          | Polyester 65%<br>Rayon 35% | 24 <sup>a</sup> | 3.1           | 0.116                         |
| 5          | Polyacrylonitrile          | ditto           | 2.7           | 0.087                         |
| 6          | Polyester 65%<br>Rayon 35% | ditto           | 4.8           | 0.189                         |

For this investigation, fabrics of the following specification were prepared on a weaving loom having a regular rotation speed of 165 RPM.

|                      |                                                              |
|----------------------|--------------------------------------------------------------|
| Fabric width         | 40 inch                                                      |
| Warp                 | Sample yarn                                                  |
| Filling              | 20 <sup>b</sup> blended yarn of 65% polyester with 35% rayon |
| Total number of warp | 4,350 ends                                                   |

From this result, it is concluded that the *S*-value of a yarn should favorably be smaller than 4.0, more favorably smaller than 3.0 in order to limit the frequency of yarn breakage within an economically acceptable range.

Example 2

Polyester staple fibers of 1.5 denier fineness and 38 mm fiber length having five kinds of differently shaped crimps were used as the material. These material fibers were manufactured into slivers of 90 grain/15 yards thickness and 0.5 TPI. by passing through an opening process, a cording process, two stayed drawing processes and a roving process. Using these slivers as specimens, values of draw-out resisting force *F<sub>D</sub>* in g and keep-in resisting force *F<sub>A</sub>* in mg were measured. Subsequent to this measurement, the slivers were processed through an open-end spinning process of the present invention and the resultant yarn breakages during the process were measured together with the thickness unevenness of the manufactured yarn. The measured results are illustrated in Table 8.

TABLE 8

| Sample No. | <i>F<sub>D</sub></i> | <i>F<sub>A</sub></i> | <i>F<sub>A</sub>-F<sub>D</sub>/NL</i> | Yarn breakage end/1000 smp. hr. | U%   | 60 |
|------------|----------------------|----------------------|---------------------------------------|---------------------------------|------|----|
| 1          | 94.3                 | 1.38                 | 0.41                                  | 380                             | 15.1 |    |
| 2          | 114.3                | 1.57                 | 0.39                                  | 540                             | 15.6 | 65 |
| 3          | 116.9                | 1.52                 | 0.31                                  | 747                             | 16.8 |    |
| 4          | 107.9                | 1.44                 | 0.33                                  | 412                             | 17.3 |    |
| 5          | 76.4                 | 1.31                 | 0.45                                  | 55                              | 13.3 |    |

As is apparently shown in the table, increase in the value of

$$\left( F_A - \frac{F_D}{NL} \right)$$

leads to decrease in yarn breakage and *U* percent.

Example 3

Measurement, the same with that taken in the preceding example, was carried out on material staple fibers of 1.5 denier fineness and 38 mm fiber length. Polyamide, polyacrylonitrile, polypropylene and rayon fibers were used as the material. The obtained result is presented in Table 9.

TABLE 9

| Sample No. | Material fiber    | <i>F<sub>D</sub></i> | <i>F<sub>A</sub></i> | <i>F<sub>A</sub>-F<sub>D</sub>/NL</i> | Yarn breakage in end/1,000 smp. hr. | <i>U</i> , percent |
|------------|-------------------|----------------------|----------------------|---------------------------------------|-------------------------------------|--------------------|
| 1          | Polyamide         | 64.3                 | 1.48                 | 0.82                                  | 12.3                                | 14.3               |
| 2          | Polyacrylonitrile | 54.6                 | 1.48                 | 0.92                                  | 32.8                                | 12.3               |
| 3          | Polypropylene     | 52.8                 | 1.41                 | 1.07                                  | 16.8                                | 11.6               |
| 4          | Rayon             | 60.3                 | 1.36                 | 0.74                                  | 29.4                                | 12.7               |

It is apparently understood from the above-presented results that the larger the value of

$$\left( F_A - \frac{F_D}{NL} \right)$$

the more uniform the yarn quality lengthwise is and the fewer frequent yarn breakages. It is further confirmed that yarn breakage of allowable frequency in the actual production process and unevenness of yarn thickness of permissible extent in the resultant textile products appearance can be desirably resulted if the value of

$$\left( F_A - \frac{F_D}{NL} \right)$$

exceeds 0.45 mg. Provision of a spinning material bundle of this nature such as a sliver or roving is easily assured by a suitably combined selection of crimp shape, crimp resiliency, oiling agent fed to the material staple fibers and lateral cross-sectional profile of a single fiber. It is also helpful, in this regard, to subject the fibrous bundle to repeated stages of a drawing process.

Example 4

Polyacrylonitrile fibrous bundles of 1.5 denier fineness and 38 mm fiber length were prepared. One of the bundles was processed through the open-end-type spinning system of the present invention and the other through the conventional ring-spinning-type system to obtain spinning yarns of 30<sup>b</sup>. The twist constant for the former was of 4.5 and that for the latter was of 3.8. Next, thusly obtained spun yarns were subjected to measurement of water retainment and the resultant percent water retainment was 167 percent for yarn manufactured by the method of the present invention and 135 percent for the yarn manufactured by the conventional ring-spinning method. The moisture content of the above used polyacrylonitrile fiber at 20° C and 65 percent relative humidity was 1.6 percent and the percent boiling water shrinkage was 2.5 percent.

From the spun yarns above-obtained, men's undershirts were manufactured in a knitting manner under the following specification.

|                                       |                                                    |
|---------------------------------------|----------------------------------------------------|
| Knitting machine used                 | Double interlock rib knitting machine of 21 gauge. |
| Number of the supplied yarns          | 20                                                 |
| Yarn speed in m./min.                 | 60                                                 |
| Yarn tension in g                     | 3                                                  |
| Diameter of the cylinder in cm        | 20                                                 |
| Rotation speed of the cylinder in RPM | 14                                                 |

The two kinds of knitted fabrics made in the above manner were passed through a bleaching treatment and subjected to quality evaluation test, the result of which is shown in the following Table 10.

TABLE 10

|                                             | Spun yarn of the invention used | Spun yarn of the conventional method used |
|---------------------------------------------|---------------------------------|-------------------------------------------|
| Weight in g./m. <sup>2</sup>                | 230                             | 227                                       |
| Thickness in mm.                            | 1.06                            | 1.00                                      |
| Degree of bulkiness in cm. <sup>3</sup> /g. | 6.10                            | 5.37                                      |
| Percent water retention                     | 213                             | 187                                       |

The listed percent water retentions were measured using test fabric pieces of 5 cm.  $\times$  5 cm. size.

It is apparent from this result that, using the spun yarn of the present invention, a knitted fabric having enhanced water retainability and particularly suitable for sweat absorption can be obtained.

Example 5

Polyethyleneterephthalate polymer having an intrinsic viscosity of 0.66 was processed through spinning, drawing and crimp impartation. The specification of the crimps imparted to the drawn filament was as follows.

|                                   |      |
|-----------------------------------|------|
| Number of crimps in 25 mm. length | 12.8 |
| Percent crimp                     | 12.0 |

After this crimp impartation, the crimped filaments were subjected to heat-set temperatures, respectively. Subsequent to these heat-set treatments, respective heat-set filaments were cut into staple fibers and processed through a mixing and blowing operation, a carding operation, two stages of drawing operations, a roving operation and a spinning operation on a spinning system shown in FIG. 1. The resultant yarn breakages in the spinning operation, yarn thickness unevenness and percent boiling water shrinkage are shown in Table 11.

TABLE 11

| Heat-set temperature in °C | Yarn Breakage in end/1000 spl. hr. | U%   | Percent boiling water shrinkage |
|----------------------------|------------------------------------|------|---------------------------------|
| 90                         | 48                                 | 13.1 | 4.7                             |
| 105                        | 55                                 | 13.3 | 3.4                             |
| 120                        | 124                                | 15.1 | 2.4                             |

One of the objects of the heat-set treatment performed here is the stabilization of the crimps already imparted to the filament. Another object of it is elimination of dependency of the shrinkability and affinity to dye of the staple fibers upon the processing conditions in the following twist-set, heat-set or dyeing operation, that is stabilization of the internal configuration of the produced spun yarns. This heat-set treatment also has a great effect upon the crimp resiliency and crimp durability of the spun yarn obtained.

Judging from this result, the preferable heat-set temperature to be employed in the art of the present invention is in a range from 100° to 115° C. When the temperature exceeds this upper limit, a considerable increase in the yarn breakage during the yarn formation and unevenness in the yarn thickness while the heat-set temperature under this lower limit will result in abnormal increase in the resultant spun yarn shrinkability. This latter increase tends to accompany difficulty in uniform dyeing of the spun yarn.

Example 6

Several kinds of staple fibers were made of polyacrylonitrile fibers having various cross-sectional profile characteristics *K* and the relationship between the value and the processing characteristics of the fibers in the spinning operation was investigated as shown in the following Table 12.

TABLE 12

| 5  | Sample No. | K     | F <sub>A</sub> in mg. | Coefficient of static friction | Coefficient of dynamic friction |
|----|------------|-------|-----------------------|--------------------------------|---------------------------------|
| 10 | 1          | 0.322 | 19.3                  | 0.436                          | 0.326                           |
|    | 2          | 0.317 | 20.1                  | 0.431                          | 0.302                           |
|    | 3          | 0.311 | 20.1                  | 0.382                          | 0.288                           |
|    | 4          | 0.304 | 21.8                  | 0.349                          | 0.280                           |
|    | 5          | 0.287 | 22.4                  | 0.339                          | 0.273                           |

15 Next, thusly prepared staple fiber samples were processed through a mixing and blowing operation, a carding operation, two-staged drawing operations and a roving operation to obtain rovings of 90 grain/15 yards thickness and of 0.5 TPI. twists. Processing these roving samples through the spinning system shown in FIG. 1, yarn breakage and resultant unevenness of the yarn thickness were measured as shown in Table 13.

TABLE 13

| 25 | Sample No. | Yarn breakage in end/1000 spl.hr. | U%   |
|----|------------|-----------------------------------|------|
| 30 | 1          | 380                               | 15.3 |
|    | 2          | 113                               | 15.1 |
|    | 3          | 97                                | 14.2 |
|    | 4          | 69                                | 13.6 |
|    | 5          | 34                                | 12.7 |

35 As is apparent from the results shown in Tables 12 and 13, increase in the value of *K* leads to increase in the keep-in resisting force *F<sub>A</sub>* in mg., decrease in the coefficients of static and dynamic frictions, decrease in yarn breakage and decrease in *U* percent. Therefore, in case of synthetic fibers of polyacrylonitrile group, favorable operational success can be obtained with decrease in the value of *K*.

40 Further, it may be well understood from the above-presented experimental results that the value of *K* should preferably be 0.3 or smaller. It was also confirmed by the inventors of the present invention that the poly-acrylonitrile group staple fibers of the above-described nature can be easily produced by adopting suitable modifications in the known synthetic filaments spinning and drawing process.

Example 7

50 Stock dyed 100 percent polyester fibers of 2 denier fineness and 51 mm fiber length were processed through the open-end-type spinning system of the invention to form a spun yarn of 24<sup>°</sup>. The yarn was provided with an average twist angle of 52.0<sup>°</sup> in its inner-layer portion. Next, men's stockings were made of the spun yarns under the following specification and the obtained stockings were subjected to a steam-set treatment for 1 minute at 110° C temperature after sewing.

| 60 | Knitting machine used            | Hosiery knitting machine of links-boss type |
|----|----------------------------------|---------------------------------------------|
|    | Diameter of the cylinder in inch | 4                                           |
|    | Number of the needles            | 176                                         |
| 65 | Supplied yarn                    | Plied yarn of two set supply                |
|    | Supply speed in m./min.          | 65                                          |
|    | Yarn tension in g./2 ends        | 3 ~ 4                                       |
|    | Texture                          | Rib stitch                                  |
|    | leg part                         | Plain stitch                                |
|    | other parts                      |                                             |

70 From thus prepared specimen knitted socks, a heel part, which requires resistance against pill formation and abrasion resistance, and a leg part, which requires extensibility, were selected and subjected to knitted fabric tests. The obtained results are shown in Table 14, wherein illustrated test results are given in the form of average values of the plain stitch parts and the rib stitch parts.

TABLE 14.

|                                                 |      |
|-------------------------------------------------|------|
| Bending strength of a single fiber in times     | 2800 |
| Degree of bulkiness in $\text{cm}^3/\text{g}$ . | 6.2  |
| Pill test result in grade                       | 3    |
| Abrasion resistance in times                    | 630  |

It was confirmed by this experimental result that the socks, which were made of material spun yarns produced by the method of the present invention, were provided with preferable resistance against pill formation and soft hand feeling due to enhanced degree of bulkiness despite their remarkably increased bending strength.

#### Comparative Example 1

Using the material fibers the same with those used in the preceding Example 7, a spun yarn of  $24^\circ$  was produced on an ordinary ring-spinning machine adapted for synthetic fiber spinning. The average twist angles of the individual fibers with respect to the yarn axis were  $52.0^\circ$  and  $22.5^\circ$ . Knitted fabrics were manufactured from these spun yarns in a manner the same with that employed in the preceding example and, after knitting operation, the fabrics were sewn into men's socks, respectively, and subjected to steam setting operations. The socks made of the spun yarns of  $52.0^\circ$  twist angle were provided with rough hand feeling and uncomfortable for wearing while the socks made of the spun yarns of  $22.5^\circ$  twist angle were provided with soft hand feeling and comfortable for wearing. Next, the two kinds of socks were subjected to the fabric test the same with that adopted in the preceding example and the results obtained are as follows.

TABLE 15.

|                                                 |      |      |
|-------------------------------------------------|------|------|
| Twist angle in degree                           | 52.0 | 22.5 |
| Bending strength of a single fiber in times     | 2800 | 2800 |
| Degree of bulkiness in $\text{cm}^3/\text{g}$ . | 5.82 | 1    |
| Abrasion resistance in times                    | 650  | 380  |

From this result, it was revealed that a trial to create a soft hand feeling inevitably accompanies deterioration in resistance against pill formation and abrasion resistance and a trial to improve the latter induces lowering of the former.

Evaluations of degree of bulkiness, abrasion strength and resistance against pill formation were carried out in the following manners.

For the evaluation of degree of bulkiness, a specimen socks cloth of  $W_g$  weight and  $A \text{ cm}^2$  surface area is subjected to a 7

$\text{g}/\text{cm}^2$  loading and the thickness  $t \text{ cm}$ . under this loaded condition is measured. In case the socks are provided with partially different textures, measurement is performed on respective parts and an average thereof is used. From the above measurement degree of bulkiness in  $\text{cm}^3/\text{g}$  is given by;

$$(At/w)$$

Evaluation of abrasion resistance is carried out following the method prescribed in ASTM. D1175-64T using a pressing load of  $1^\circ$ , pneumatic pressure of  $4^\circ\text{lb}/\text{in}^2$  and an abrasive paper of CC800-CW type.

Evaluation of resistance against pill formation is carried out on an ICI-type pill tester.

What is claimed is:

1. An improved spun yarn comprising an inner fibrous layer and an outer fibrous layer with no distinct boundary between said layers, the number of twist possessed by fibers of said outer layer being different from that possessed by fibers of said inner layer with respect to a central longitudinal axis of said spun yarn, the spiral diameter of every fiber composing said yarn being substantially identical, the value of unevenness index not exceeding 10 and the value of variations of stretching tension not exceeding 4.
2. An improved spun yarn according to claim 1, in which said fibers composing said spun yarn are staple fibers having a moisture content not exceeding 4.1 percent and the percent of water retention of said spun yarn being not less than 150 percent.
3. A textile product made up of spun yarns claimed in claim 1 and having a degree of bulkiness ranging from 6.0 to 7.0  $\text{cm}^3/\text{g}$ .
4. A textile product made up of spun yarns claimed in claim 2 and having degree of bulkiness ranging from 6.0 to 7.0  $\text{cm}^3/\text{g}$ .

5. A method of manufacturing an improved spun yarn on an open-end-type spinning system having a fiber strand feeding device, a spinning rotor rotating at high speed and a take-up device, characterized by supplying to said feeding device a fiber strand of the following characteristics  $F_A - (F_D/NL) > 0.45$

wherein:

$$F_A = \text{Keep-in resisting force}$$

$$F_D = \text{Draw-out resisting force}$$

$N$  = Number of individual fibers contained in a cross-section of said strand

$L$  = Average fiber length in mm,

the fibers of said strand are drawn out of said feeding device, transported pneumatically to the interior of said spinning rotor and therein twisted into a yarn which is delivered to take-up device.

6. A method according to claim 5, in which said supplied fiber strand is composed of staple fibers having a cross-sectional profile characteristic not exceeding 0.3.

\* \* \* \* \*